

1

3,574,049

### TRANSFER PRINTING

Pierre Sander, Tourcoing, France, assignor to  
Trentesaux-Toulemonde, Tourcoing, France  
No Drawing. Filed Mar. 14, 1967, Ser. No. 623,045  
Claims priority, application France, Mar. 16, 1966,  
53,596

Int. Cl. B32b 15/20, 23/22, 29/00  
U.S. Cl. 161—220

6 Claims

### ABSTRACT OF THE DISCLOSURE

A temporary support for transfer printing, which consists of a member selected from a sheet of paper and an aluminum foil coated on one of its faces with a transfer coating of ethylcellulose which bears a pigmented film of a resin selected from the group consisting of the thermoplastic polyamide and vinyl resins.

This invention relates to transfer printing, especially on plastics materials.

A transfer printing process has already been proposed in which a design is fixed to a temporary support by means of an adhesive and in which, after being soaked in water this design is applied to a final support where it remains when the temporary support is removed.

It has also been proposed to print designs on a temporary support using water inks and then to transfer the said designs by bringing a final support, which has been previously moistened, into contact with them.

In another process it has been proposed to transfer designs by applying heat. In this process the coloring materials, for example, inks, penetrate into the body of a temporary support made of paper and sublime on heating to high temperatures to condense on the material which forms a final support.

In other processes, it has been proposed to replace the adhesives on the temporary support by waxes or soft resins, onto which the designs to be transferred are printed. Just as, when water transfers are used, a residue of adhesive often remains on the final support, so in these processes, the waxes and soft resins are often transferred at the same time as the design onto the article to be printed. The result is that the printed article has a greasy appearance which is not always desired and also that the fixing of the inks of the design is not certain. The resulting designs look dull and offer little resistance to destructive agents and to weathering.

Processes which make it possible to produce hot marking on numerous materials have been proposed, for example, the process known by the name of "Roll Leaf" in the United States and the process known under the name of "Blocking Foil" in Great Britain. Such processes have the disadvantage that they also fix a part of a film detached from the temporary support onto the final support of the print. The presence of such a piece of film, which is generally glossy and covers more than the entire transferred design, is not always desirable.

Particularly in the field of synthetic plastics, films on which designs in several colors are to be printed have to pass through machines provided with inking stations arranged around a cylinder and may, as a result of their inherent elasticity, have to be held on a relatively inextensible adhesive belt whilst passing through the machine.

While such devices keep the material to be printed steady, it is not possible to have large drying distances between the printing positions for the different colours and as a result it is necessary to work at very slow speeds. The resulting transfer is of poor quality, and often unsatisfactory. When dealing with prints on non-planar surfaces, for example the surfaces of moulded articles, the

2

multicolor prints have to be effected color by color. Such processes take a very long time.

The present invention overcomes the disadvantages of the proposed processes and makes it possible to print 5 multi-color designs onto articles which have been hitherto difficult to print on account of their shape, and/or their physicochemical or mechanical properties.

The present invention provides a transfer process for printing a design on a final support which comprises (a) 10 printing a design onto a temporary support, (b) superimposing the temporary support and the final support, (c) applying heat and/or pressure to the superimposed structure formed in (b), and (d) separating the temporary support from the final support which retains the printed design, the affinity of the material of the design 15 for the temporary support being lower than its affinity for the final support.

Advantageously, when heat is applied in step (c) of the process of the invention, the superimposed structure 20 is allowed to cool before the temporary support is separated from the final support. Pressure may be applied to the superimposed structure in step (c) by, for example, passing it between cylinder rollers, by calendering or by pressing it between plates.

Preferably, the difference between the affinity of the material of the design for the temporary support and its affinity for the final support increases with increasing temperature.

The temporary support may comprise a coating, called 30 a transfer coating, of a material for which the material of the design has an affinity lower than its affinity for the final support, and preferably the difference between the two affinities also increases with increasing temperature.

The designs transferred may be of any color or size. 35 They may be printed on the temporary support by any known technique, for example, by rotogravure, offset or flexographic printing.

Designs may be printed on the front and the back of 40 a final support which is in the form of a sheet by applying two temporary support sheets to the respective faces of the final support in the process of the invention. On final supports which are transparent, translucent or opalescent it is possible to obtain a front and a back print of one and the same object inverted, making it possible to achieve 45 a depth effect.

The transfer process of the invention makes it possible 50 to print final supports whose rigidity, or lack of rigidity, makes them unsuitable for passing through a normal printing machine. There is no relative movement between the temporary support and the final support whilst the transfer is being made.

In a particular form of the process of the present invention, the design may be transferred during the manufacture of the final support itself. This is the case when 55 the final support is made from a plastisol. The plastisol is spread onto the previously printed temporary support and during the gelling of the plastisol the design is completely transferred to the final support. Thus, particularly for moulded articles, the transfer may be carried out by 60 incorporating the temporary support, in the form of, for example, a label, in the mould itself before moulding.

Whether or not the temporary support comprises a transfer coating, a protective varnish may be applied to the temporary support, optionally only to certain parts 65 of it, before the temporary support is printed with the design in step (a) of the process of the invention, the affinities of the protective varnish and the material of the design for the temporary support being similar and the affinities of the protective varnish and the material of the 70 design for the final support being similar, so that the varnish is transferred to the final support together with the design during the transfer process.

Such a protective varnish may be, for example, a synthetic resin in emulsion form. The presence of a layer of protective varnish gives the transferred designs excellent resistance to abrasion, dissolution, weathering and other causes of destruction. The use of emulsions makes it possible to apply heavier coatings giving superior mechanical properties.

The inks of the designs should be adapted to the properties of the materials of the final supports. They should contain colorants which do not migrate into the final support, which have good fastness to light and which, when colors are to be superimposed, are transparent, so that the shades obtained after transfer are not changed because of the opacity of one or more of the constituent colorants. On the other hand, when transfer onto a transparent final support is desired, the transferred designs can be rendered opaque by printing a white ink as a last layer onto the designs carried by the temporary support.

The process of the present invention is particularly suited to the transference of designs onto final supports of polyvinyl chloride or polypropylene or of polyethylene. In such cases, especially when vinyl resins are used as bases for the inks which form the desired designs, it is advantageous to use a temporary support comprising a transfer coating of ethyl cellulose, which is practically incompatible with said vinyl resins. The transfer coating may also comprise up to 10% by weight of octyl adipate to give the transfer coating sufficient coherence to receive a multicolored design by the printing technique employed.

The support for the ethyl cellulose transfer coating is preferably substantially dimensionally stable to heat. It may be, for example, a sheet of thick aluminum foil, or a sheet of non-porous paper, or a sheet of thin aluminum foil optionally backed with paper, with a cellulosic film or with a plastic film of, for example, polyethylene or polypropylene.

Generally the thickness of the ethyl cellulose transfer coating is such that from 0.5 to 5 gms. of ethyl cellulose covers one square metre of the surface of the temporary support.

The inks which form the designs may have, for example, the following composition by weight:

| Colorant           | Parts |
|--------------------|-------|
| Vinyl resin        | 12    |
| Toluene            | 6     |
| Methylethyl ketone | 10    |
|                    | 72    |



As colorants, those known by the name of "Microlithe K" are especially suitable. These are fine dispersions of pigments in thermoplastic resins, for example, vinyl resins, and absolutely transparent prints may be obtained using them. The pigments themselves are generally organic materials, for example, azo pigments obtained by coupling or condensation, anthraquinone colorants, perinones or perlyenes, quinacridones, thioindigo, dioxazines or phthalocyanines. French patent specification No. 1,079,477 described "Microlithe K" colorants containing one or more compounds of the formulae



5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

805

810

815

820

825

830

835

840

845

850

855

860

865

870

875

880

885

890

895

900

905

910

915

920

925

930

935

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

5

which had been prepared by mixing 8 parts of a 40% dispersion of a compound of the formula



in the copolymer of vinyl chloride and vinyl acetate described in Example 1, together with 2 parts of a 45% dispersion of a compound of the formula



in the aforesaid copolymer, 5 parts of the aforesaid copolymer, 5 parts of "Kunstharz AFS," 10 parts of toluene and 68 parts of methyl ethyl ketone.

### EXAMPLE 3

A temporary support prepared as in Exemple 1 was printed with a design using an ink of the composition,

(a)

|                                                                                                                        | Percent |
|------------------------------------------------------------------------------------------------------------------------|---------|
| Aluminum "Microlithe K" (finely powdered aluminum coated with a copolymer of 85% vinyl chloride and 15% vinyl acetate) | 15      |
| Vinylite VMCH resin                                                                                                    | 7       |
| Toluene                                                                                                                | 10      |
| Methyl ethyl ketone                                                                                                    | 68      |

followed by an ink of the composition

(b)

|                                   | Percent |
|-----------------------------------|---------|
| "Microlithe K" Blue and/or Yellow | 12      |
| Vinylite VMCH resin               | 6       |
| Toluene                           | 10      |
| Methyl ethyl ketone               | 72      |

On completing the transfer process as in Example 1, a polyvinyl chloride sheet was obtained having a metallic-colored design on one face.

#### EXAMPLE 4

A temporary support prepared as in Example 1 was printed with a design using an ink of the composition,

|                                        | Percent |
|----------------------------------------|---------|
| "Microlithe K" Yellow, Red or Blue     | 12      |
| Vinylite VMCH resin                    | 6       |
| Toluene                                | 10      |
| Methyl ethyl ketone                    | 72      |
| followed by an ink of the composition, |         |
| Titanium dioxide                       | 10      |
| Rhodopas AX                            | 10      |
| Vinylite VMCH resin                    | 6       |
| Toluene                                | 10      |
| Methyl ethyl ketone                    | 64      |

On completing the transfer process as described in Example 1, only in this case using a transparent polyvinyl 75

6

chloride sheet, a non-transparent colored design was transferred onto the transparent polyvinyl chloride sheet.

**EXAMPLE 5**

- 5 A face of an aluminum sheet, thickness 6.5 microns, was coated with the following composition:

|                                           | Percent |
|-------------------------------------------|---------|
| Ethyl cellulose (20 cps. viscosity) ----- | 10      |
| Octyl adipate -----                       | 1       |
| 95% ethyl alcohol -----                   | 89      |

so that, after evaporation of the ethyl alcohol, a coating of 6 gms./sq. metre of ethyl cellulose remained.

15 The coated face was then printed with a design, by means of an inking roller using ink which had been prepared as follows:

20 parts of a 50% dispersion of the colorant of the formula

20



in the polyamide resin known under the trade name Vers-  
40 amide 930 (a dispersion in which the average particle size  
was less than 0.5 micron) were mixed, with good stirring,  
with 10 parts of the aforesaid resin, 35 parts of n-octane  
and 35 parts of isopropyl alcohol.

After drying, an aluminum film having on one of its faces, a design layer separated from the metallic surface by ethyl cellulose was obtained.

This printed temporary support was superimposed on a sheet, or a cylinder or any object of polyethylene. After heating of the superimposed structure under gentle pressure, the aluminum foil together with its transfer coating of ethyl cellulose was peeled off leaving the design firmly transferred to the polyethylene.

I claim:

- 55 1. A temporary support for transfer printing, which consists of a member selected from a sheet of paper and an aluminum foil which member is coated on one of its faces with a transfer coating of ethylcellulose which bears a pigmented film of vinyl chloride polymers or copolymers.

60 2. A temporary support as claimed in claim 1, which consist of an aluminum sheet backed on one of its faces with paper, and bearing on the other face a coating of ethyl cellulose covered with a multicolored film consisting essentially of a copolymer of vinylchloride and vinylacetate.

65 3. A temporary support as claimed in claim 1, wherein the pigmented film is of polyvinylchloride.

70 4. A temporary support as claimed in claim 1, wherein the transfer coating comprises from 0.5 to 6 gms. of ethyl cellulose per square metre.

75 5. A temporary support as claimed in claim 1, wherein the transfer coating comprises from 0.5 to 6 gms. of ethyl cellulose per square metre and has been printed with a layer of a design of pigmented polyvinylchloride.

80 6. A temporary support as claimed in claim 5, wherein

the design layer is transparent and has a thickness of 90 to 900 microns.

3,265,524 8/1966 Echeagaray ----- 161—220  
3,298,850 1/1967 Reed ----- 117—3.1

## References Cited

## UNITED STATES PATENTS

|           |         |                 |          |    |                                                    |
|-----------|---------|-----------------|----------|----|----------------------------------------------------|
| 3,013,918 | 12/1961 | Betham -----    | 161—268X | 5  | JOHN T. GOOLKASIAN, Primary Examiner               |
| 2,746,877 | 5/1956  | Matthews -----  | 117—3.1  |    | L. T. KENDELL, Assistant Examiner                  |
| 2,990,311 | 6/1961  | Shepherd -----  | 161—249  |    | U.S. Cl. X.R.                                      |
| 3,014,828 | 12/1961 | Reese -----     | 161—406  |    | 117—3.1, 73, 127, 157; 156—230, 234, 309; 161—249, |
| 3,031,324 | 4/1962  | Jankowski ----- | 117—3.1  | 10 | 268, 406, 413                                      |
| 3,065,120 | 11/1962 | Avelar -----    | 117—3.1  |    |                                                    |